

# United States Patent Office.

WILLIAM PYLE, OF WILMINGTON, DELAWARE.

*Letters Patent No. 105,247, dated July 12, 1870.*

## IMPROVEMENT IN THE MANUFACTURE OF LEATHER.

*The Schedule referred to in these Letters Patent and making part of the same.*

*To all whom it may concern:*

Be it known that I, WILLIAM PYLE, of the city of Wilmington, in the State of Delaware, leather manufacturer, have invented a new and useful Improvement in the Manufacture of Leather; and I do hereby declare the following to be a full and correct description of the same.

My invention consists in a new process or method of treating buff leather, so as to produce an article having a close resemblance, in appearance and qualities, to morocco, and applicable to the manufacture of shoes and to other purposes for which morocco is employed, and which is not liable to crack or wear white, as the ordinary patent leather does. The essence of the invention lies in the order and the character of the applications to the leather.

The ordinary patent leather is made by the application of a heavy coat of varnish or composition to the buff leather, and, being finished dry, with no oil, it will crack in cold weather, and is not well suited for shoe-leather on that account, and because it wears white, owing to the varnish being applied to undyed stock.

My process is as follows:

After buffing I dye the leather of the desired color. By reason of the color being thus applied before the finishing composition, a much thinner coating of the latter is required in order to cover, and the composition, when worn off, does not disclose a white surface below it.

After dyeing I apply a composition, consisting of linseed-oil thinned with benzine, and containing appropriate coloring matter. I lay this composition on with a brush in very thin coats, so thin as entirely to prevent that hardening of the leather which occurs in the ordinary manufacture of patent leather. My coating dries in about one day, thus saving three or four days over the common process in the drying alone. I next oil the leather on the flesh side, and wet it before graining. I then grain wet, getting a fine pebbly surface, and finish by oiling, giving the leather almost the exact appearance of morocco, and making it soft and pliable, and suited for the manufacture of shoes. It is more durable than morocco.

Having thus fully described my invention—

What I claim, and desire to secure by Letters Patent, is—

The process or method hereinbefore described of manufacturing buff leather in imitation of morocco by dyeing the leather after buffing, then applying the surface composition, and, finally graining wet and oiling, all in the order and manner set forth.

The above specification of my said invention signed and witnessed at Wilmington this 17th day of May, A. D. 1870.

WM. PYLE.

Witnesses:

W. H. CLOWARD,  
JOSEPH PYLE.